

Patented June 10, 1924.

## UNITED STATES PATENT OFFICE.

HARRY P. BASSETT, OF CYNTHIANA, KENTUCKY, AND THOMAS F. BANIGAN, OF  
PHILADELPHIA, PENNSYLVANIA.

## PROCESS OF MAKING ARTIFICIAL SILK AND SIMILAR PRODUCTS.

No Drawing.

Application filed May 14, 1923. Serial No. 638,950.

*To all whom it may concern:*

Be it known that we, HARRY P. BASSETT and THOMAS F. BANIGAN, citizens of the United States, residing at Cynthiana, in the county of Harrison and State of Kentucky, and Philadelphia, in the county of Philadelphia and State of Pennsylvania, respectively, have invented certain new and useful Improvements in Processes of Making Artificial Silk and Similar Products, of which the following is a specification.

This invention relates to the production of artificial silk and has particular reference to an improved process of spinning artificial silk from a solution of a cellulose compound containing one or more acetyl radicals and one or more nitro radicals combined with the cellulose radical in one and the same compound.

We have discovered that important advantages are obtained by dissolving such acetyl nitro cellulose in a suitable quantity of a mixture of strong acetic acid, preferably glacial acetic acid, and acetone and spinning the silk from such solution. One advantage is that the resulting filaments are strong and uniform in thickness as compared with filaments spun from a solution of the same cellulose composition in some other solvent, as for example, acetone. Another advantage is that the filament is nearer round and less ribbon like in form than if spun from a solution in some other solvent. A further advantage is that by varying the proportions of the acetic acid and acetone it is possible to vary the fineness of the filament when spun from the same spinneret.

The solvent may contain from about equal volumes of strong acetic acid and acetone to about 10 parts by volume of strong acetic acid to 90 parts of acetone, it being understood that strong acetic, preferably glacial acetic acid, must be used. If acetic acid containing any considerable amount of water, as for example 5 or 10 per cent of water is used, a proportion approximating equal parts of the acetic acid and acetone is not satisfactory as the water has a pronounced precipitating effect upon the cellulose compound. Where the proportion of the acetone is materially in excess of that of the acetic acid it is possible to use acetic acid containing a substantial amount, as for example 10 to 15 per cent of water. We

prefer, however, in all cases, to use acetic acid containing not more than about 5 per cent of water and we ordinarily prefer to use glacial acetic acid to avoid the precipitating action of water in the solvent since the greater the percentage of water therein the greater must be the proportion of the acetone to the acetic acid to overcome the precipitating effect of the water.

In practice in spinning artificial silk for ordinary usage, such for example as for use in the manufacture of ordinary hosiery, dress fabrics, knit goods, and the like, we prefer to spin the acetyl nitro cellulose from a solution in about 3 parts by volume of glacial acetic acid to 7 parts by volume of acetone. For making very fine filaments for use in making the highest grade of silk fabric in which a very high degree of softness, flexibility, and resemblance to natural silk are to be obtained, we prefer to spin the acetyl nitro cellulose from solution in a mixture of about 3 parts by volume of glacial acetic acid to 17 parts by volume of acetone. Our spinning solution ordinarily contains from 8 to 12 per cent by weight of the acetyl nitro cellulose depending upon whether the silk is to be fine, soft and lofty or strong and of a lesser degree of fineness, softness and loftiness, the higher the percentage of the cellulose composition in the spinning solution the stronger and less fine, soft and lofty will be the fabric produced from the resulting filaments. It will be understood by those skilled in this art that the percentage of cellulose composition in the spinning solution may be materially above and materially below the range which we ordinarily employ. For example, we may spin from a solution containing as low as about 5 per cent and as high as about 15 per cent by weight of the cellulose composition, the percentages which we ordinarily use as indicated above are however preferred.

While our improved artificial silk can be dry spun from solution in the solvent hereinbefore described we have found it to be advantageous to spin it into a solution which will immediately absorb the acetone from the filament as it issues from the spinneret but which will not wholly remove the acetic acid, it having been found that it is desirable to have the filament under the influence of the acetic acid until it is given its

final form. This is particularly advantageous in spinning very fine filaments such for example as filaments of 50 to 75 deniers for a thread of 18 filaments. To accomplish this purpose we prefer to spin our filaments preferably upwardly, into dilute acetic acid of from about 10 to 50 per cent strength and we prefer to use acid of about 30 per cent strength.

10 It will be understood that our process is adapted for use in making artificial horse hair, artificial straw and other forms of cellulose bodies which are formed by forcing plastic cellulose material through a shaping orifice.

15 While we have described in detail the preferred practice of our process and the preferred proportions of reagents it is to be understood that the details of procedure of such process and the proportion of materials used may be varied within the scope of the subjoined claims without departure from the spirit of our invention.

Having described our invention, we claim:

20 1. The herein described process of making artificial silk, artificial horse hair, artificial straw and the like which consists in dissolving a cellulose composition containing both acetyl and nitro groups combined with cellulose in a single compound in a mixture of strong acetic acid and acetone to form a spinning solution and forcing the spinning solution through a shaping orifice.

25 2. The herein described process of making artificial silk, artificial horse hair, artificial straw and the like which consists in dissolving a cellulose composition containing both acetyl and nitro groups combined with cellulose in a single compound in a mixture of about from 10 to 50 parts by volume of strong acetic acid to 50 to 90 parts by volume of acetone to form a spinning solution and forcing the spinning solution through a shaping orifice.

30 3. The herein described process of making artificial silk, artificial horse hair, artificial straw and the like which consists in dissolving a cellulose composition containing both acetyl and nitro groups combined with cellulose in a single compound in a mixture of about from 10 to 50 parts by volume of glacial acetic acid to 50 to 90 parts by volume of acetone to form a spinning solution

and forcing the spinning solution through a shaping orifice.

4. The herein described process of making artificial silk, artificial horse hair, artificial straw and the like which consists in dissolving a cellulose composition containing both acetyl and nitro groups combined with cellulose in a single compound in a mixture of strong acetic acid and acetone to form a spinning solution, and forcing the spinning solution through a shaping orifice into a liquid adapted to withdraw the acetone therefrom without wholly withdrawing the acetic acid.

5. The herein described process of making artificial silk, artificial horse hair, artificial straw and the like which consists in dissolving a cellulose composition containing both acetyl and nitro groups combined with cellulose in a single compound in a mixture of strong acetic acid and acetone to form a spinning solution and forcing the spinning solution through a shaping orifice into a solution of dilute acetic acid.

6. The herein described process of making artificial silk, artificial horse hair, artificial straw and the like which consists in dissolving a cellulose composition containing both acetyl and nitro groups combined with cellulose in a single compound in a mixture of strong acetic acid and acetone to form a spinning solution and forcing the spinning solution through a shaping orifice into a solution of dilute acetic acid of about from 10 to 50 per cent strength.

7. The herein described process of making artificial silk, artificial horse hair, artificial straw and the like which consists in dissolving a cellulose composition containing both acetyl and nitro groups combined with cellulose in a single compound in a mixture of strong acetic acid and acetone to form a spinning solution and forcing the spinning solution through a shaping orifice into a solution of dilute acetic acid, of about 30 per cent strength.

In testimony whereof we affix our signatures in presence of two witnesses.

HARRY P. BASSETT.  
THOMAS F. BANIGAN.

Witnesses:

EVA ROBERTS,  
D. R. ARCHIBALD.